

# United States Patent Office

2,881,202

Patented Apr. 7, 1959

1

2,881,202

## GASOLINE IGNITION CONTROL ADDITIVES

John A. Pianfetti, South Charleston, W. Va., and Gen-  
nady M. Kosolapoff, Auburn, Ala., assignors to Food  
Machinery and Chemical Corporation, New York,  
N.Y., a corporation of Delaware

No Drawing. Application October 7, 1955  
Serial No. 539,259

6 Claims. (Cl. 260—461)

This invention relates to new compositions of matter, 15  
their novel preparation and their use as gasoline igni-  
tion control additives.

More particularly, this invention relates to organophosphorous compounds as new compositions of matter, their 20  
novel preparation and their use as gasoline ignition con-  
trol additives.

The need for improved gasolines has been spurred since  
the end of World War II by the automotive industry's race  
to produce more and more powerful internal combustion  
engines. To achieve this greater horsepower, engine man-  
ufacturers have steadily increased cylinder compression  
ratios to the point where they now average 7.5 to 1. One  
of the factors necessary to achieve maximum operating  
efficiency from these high compression engines is that  
the ignition of the fuel-air mixture takes place at the mo-  
ment of greatest compression.

As engines become more powerful, they demand higher  
octane fuel which can be manufactured only with an in-  
crease in the tetra-alkyl lead content. The use of these  
organic lead compounds in gasolines leads to the forma-  
tion, during combustion, of lead salts which catalyze the  
oxidation of the carbonaceous residues from the fuel and  
oil and lower the ignition temperature of the carbon resi-  
dues thus creating glowing particles that ignite the fuel-  
air charge prematurely.

It has been the practice of the art to add to fuels con-  
taining organic lead compounds, a halohydrocarbon for  
the purpose of converting the lead into lead halides volatile  
at the combustion temperature of the gas within the  
cylinder and which lead compound would be swept out  
with the exhaust gases. These compounds are known as  
scavengers. In actual practice, however, the formation  
of lead oxyhalides and lead oxides as well as the volatile  
lead halides cannot be avoided and deposits of lead com-  
pounds are found in the combustion chamber even when  
such scavengers are employed.

It is an object of the instant invention to provide new  
compositions of matter which may be employed as gaso-  
line additives. It is another object of this invention to  
provide new compositions of matter which will aid in the  
suppression of the pre-ignition characteristics of the fuel-  
air mixture. It is a further object of this invention to  
provide novel means for preparing these new compositions  
of matter. Further objects will appear as a description  
of this invention unfolds.

We have discovered certain organophosphorous com-  
pounds having properties which render them suitable for  
use as pre-ignition control additives. It has been found  
that the defect of pre-ignition arising from the use of con-  
ventional leaded gasolines can be substantially lessened  
by the use of the compounds of this invention. These  
organophosphorous compounds appear to function by con-  
verting the lead present in the fuel into lead compounds  
having a very low catalytic effect in reducing the ignition  
temperature of the carbon deposits within the combustion  
chamber as compared to the lead compounds that form in  
the combustion chamber, absent the organophosphorous

2

compounds of this invention. Thus, an increase in the  
ignition temperature of the cylinder deposit would like-  
wise decrease the tendency of the deposit to pre-ignite the  
fuel-air mixture.

5 The terms, ignition temperature and glow point, are  
meant to be synonymous for the purposes of this specifi-  
cation unless a contrary intention is shown.

The organophosphorous compounds which we have dis-  
covered as suitable for use in accordance with this inven-  
tion are:

(1) Halogenated esters of phosphorous acid



in which R may be a hydrogen, an aliphatic chain up to  
and including six carbon members, a phenyl or substituted  
phenyl radical, X may be a member of the halogen group  
and Y may be an aliphatic chain up to and including six  
carbon members, an aryl or a substituted aryl radical.

(2) Halogenated thio esters of primary phosphonic  
acids



in which R may be a hydrogen, an aliphatic chain up to  
and including six carbon members, a phenyl or substituted  
phenyl radical, X may be a member of the halogen group  
and Y may be an aliphatic chain up to and including six  
carbon members, an aryl or a substituted aryl radical.

These new compounds, both the halogenated esters of  
phosphorous acid and the halogenated thio esters of phos-  
phonic acid, were prepared in a novel manner.

The novel manner of preparing the halogenated esters  
of phosphorous acid is through the reaction of dihalo-  
phosphines and oxiranes or substituted oxiranes.

The term oxirane is used to designate the grouping,



45 hence,



50 is known as methyl oxirane. This compound is also  
known as propylene oxide.

The aliphatic and aromatic dihalophosphines may be  
prepared by heating phosphorus trihalide with the corre-  
sponding dialkylmercury or diarylmercury derivatives in  
55 sealed tubes for several hours at 180° to 230° C., as  
described in the literature.

The examples that follow illustrate the novel prepara-  
tion of the haloesters of phosphorous acid.

## EXAMPLE 1

The apparatus used for this experiment was a 3-necked  
flask fitted with a stirrer, thermowell, reflux condenser,  
and a calibrated addition funnel.

60 The flask was charged with 179 parts of phenyl dichloro-  
phosphine. From the calibrated addition funnel was  
65 added 116 parts of methyl oxirane (propylene oxide).  
The oxirane was added over a period of an hour while  
maintaining the temperature of the reaction mass at about  
70 25° C. Upon completing the addition of the oxirane, the  
pressure in the system was reduced for a short interval  
of time to 2. mm. Hg in order to remove any traces of  
unreacted oxirane.

## 3

The product, bis(chloropropyl) phenyl phosphonite, obtained in near quantitative yield had a specific gravity of 1.180 35/4 and a refractive index of 1.5308, D/25.

Calculated for  $C_{12}H_{17}O_2PCl_2$ : P=10.5%, Cl=24.1%. Found: P=10.2%, Cl=23.4%.

## EXAMPLE 2

The apparatus used for this experiment was the same as described in Example 1.

The flask was charged with 117 parts of methyl dichlorophosphine. From the calibrated addition funnel was added 116 parts of methyl oxirane (propylene oxide). The oxirane was added over a period of an hour while maintaining the temperature of the reaction mass at about 25° C. Upon completing the addition of the oxirane, the pressure in the system was reduced for a short interval of time to 2 mm. Hg in order to remove any traces of unreacted oxirane.

The product, bis(chloropropyl) methyl phosphonite, obtained in near quantitative yield, had a specific gravity of 1.137 35/4° C. and a refractive index of 1.4638 D/25° C.

Calculated for  $C_7H_{15}O_2PCl_2$ : P=13.3%, Cl=30.4%. Found: P=12.9%, Cl=29.6%.

The novel method of preparing the halogenated thionoesters of primary phosphonic acids is by the reaction of the halogenated esters of phosphorous acid and sulphur to yield the appropriate thionophosphonate.

The examples that follow illustrate the novel preparation of the halogenated thionoesters of phosphonic acid.

## EXAMPLE 3

The apparatus used for this experiment was a 3-necked flask fitted with a stirrer, thermowell and a reflux condenser.

The flask was charged with 132 parts of bis(chloropropyl) phenyl phosphonite. After heating the phosphonite to about 80° C., 15 parts of sulphur were added slowly over a 30 minute period while keeping the temperature at about 80° C. This temperature was maintained until but a trace of sulphur remained. The product was cooled, and filtered. The product, bis(chloropropyl) phenyl thionophosphonate obtained in near quantitative yield, had a specific gravity of 1.237 35/4° C. and a refractive index of 1.5451 D/25° C.

Calculated for  $C_{12}H_{17}O_2PSCl_2$ : P=9.5%, Cl=21.7%, S=9.8%. Found: P=9.1%, Cl=21.5%, S=9.8%.

## EXAMPLE 4

The apparatus used for this experiment was the same as described in Example 3.

The flask was charged with 105 parts of bis(chloropropyl) methyl phosphonite. After heating the phosphonite to about 80° C., 15 parts of sulphur were added slowly over a 30 minute period while keeping the temperature at about 80° C. This temperature was maintained until all but a trace of sulphur remained. The product was cooled, and filtered.

The product, bis(chloropropyl) methyl thionophosphonate, obtained in near quantitative yield had a specific gravity of 1.220 35/4° C. and a refractive index of 1.4933 D/25° C.

Calculated for  $C_7H_{15}O_2PSCl_2$ : P=11.7%, Cl=26.8%, S=12.1%. Found: P=11.3%, Cl=26.5%, S=12.1%.

The reaction between the dihalophosphine and oxirane may be conducted at temperatures below the preferred temperature of 20°-40° C. The maximum temperature of reaction is that at which rearrangement of product occurs.

The reaction between the dihalophosphine and oxirane may be run at sub- or super-atmospheric pressure but for convenience it is preferable to operate at atmospheric pressure.

An inert gas, such as, carbon dioxide or nitrogen, may be passed through the system during the reaction period.

## 4

though it is not necessary to the practice of this invention that an inert atmosphere be maintained during the reaction of the dihalophosphine and oxirane.

The conversion of the haloester of phosphorous acid to the halogenated thio ester of a primary phosphonic acid by the addition of sulphur to the former may be run over a wide temperature range though it is preferable to maintain the reaction temperature at about 80° C.

Preliminary testing of these compounds as pre-ignition additives involved the common gasoline acceptance tests including: solubility of compound in gasoline, water tolerance, gum formation and copper corrosion.

The first test, gasoline solubility, was conducted to determine at least qualitatively whether the organophosphorus compounds were soluble in gasoline. This determination was made by measuring the light transmittancy of the gasoline both with and without the addition of the organophosphorus compound.

Solutions which contained 0.03 volume percent of the phosphorus compounds were prepared by adding 0.03 ml. of the compound to 100 ml. of a premium gasoline. After a short shaking and standing period the solution was transferred to an optical cell and the light transmittance of the solution measured. This value was compared to the value for the premium gasoline which did not contain an additive. A decrease in the light transmittance of the base fuel of 1% or more indicates that the additive is sufficiently soluble for the purposes of this invention.

The water tolerance was determined by following the procedure detailed in ASTM D1094-52.

The gum formation was determined by employing the copper dish method set forth in ASTM D910-52T, Section 9J.

The copper corrosion test was conducted in accordance with the instructions stated in ASTM D130-53T.

The results of the above tests are tabulated in Table I.

Illustrative of the compounds tested are bis(chloropropyl) methyl phosphonite, BCPMP; bis(chloropropyl) phenyl phosphonite, BCPPP; bis(chloropropyl) methyl thionophosphonate, BCPMTP; and tricresyl phosphate, TCP.

The inclusion of the compound, tricresyl phosphate, in the tables of the instant specification is for the purpose of comparing the compounds of the instant invention with that of a known gasoline pre-ignition additive.

Table I

| Additive | Solubility | Water tolerance | Gum formation, mg/100 ml. | Copper corrosion, ASTM index, additive conc. |        |
|----------|------------|-----------------|---------------------------|----------------------------------------------|--------|
|          |            |                 |                           | 0.03%                                        | 0.015% |
| BCPMP    | OK         | OK              | 3                         | 1                                            | -----  |
| BCPPP    | OK         | OK              | 6                         | -----                                        | 0      |
| BOPMTP   | OK         | OK              | 5                         | 1-2                                          | 0      |
| TCP      | -----      | -----           | 33                        | 0                                            | -----  |

Table I shows the compounds of the instant invention to be compatible with gasoline in so far as the common acceptance tests are concerned.

The low gum formation of the compounds of the instant invention make them particularly suitable as additives for internal combustion engines.

Compounds found satisfactory as regards the common gasoline acceptance tests were then evaluated as pre-ignition depressants.

A method, familiar to those skilled in the art for determining a compound's ability to reduce the pre-ignition characteristics of a gasoline, is the oven-test method. Broadly stated, this procedure entails placing known amounts of synthetic engine deposit in a Pyrex heating boat, with or without the pre-ignition depressant added, and having a means for measuring the temperature of the deposit connected thereto. The boats are placed in an

oven and the temperature is increased at a uniform rate. The degree of temperature resulting from a sudden increase in temperature is taken as the glow point of the deposit.

The detailed method employed in determining the glow point of the compounds of this invention is set forth below.

A synthetic engine deposit which contained 38.3% lead sulfate, 33.1% lead oxide, 7.7% lead chloride, 5.9% lead bromide and 15.0% carbon black was prepared by adding the approximate amounts of the compounds together and mixing in a mortar and pestle. To a Pyrex Petrie dish,  $\frac{9}{10}$  in. high and  $5\frac{1}{2}$  in. in diameter was added 0.40 g.  $\pm 0.1$  g. of the synthetic deposit. Over this was burned in 100 ml. portions, gasoline which contained 0.03 volume percent of the different organophosphorus compounds. The amount of additive used was dependent on the phosphorus content of the organophosphorus compound. Enough phosphorus was used to theoretically convert all the lead in the synthetic deposit to lead phosphate. Air was introduced into the gasoline during the burning operation at 2500 cc. a minute in an attempt to convert some of the carbon given off during burning to oxides of carbon. An iron-constant in thermocouple was also placed in the burning fuel in order to obtain some idea as to the temperatures that occurred in the burning step. The majority of the gasoline burned between 150-200° C. and the end gases, approximately 5-10%, burned between 350 and 450° C. After burning was finished the deposit was scraped from the bottom and the inside wall of the dish and this material then mixed in a mortar and pestle. A glow point determination was then made on the treated deposit.

The apparatus for measuring the glow point consisted of a copper block, 3 in. in length by 2 in. in diameter. A  $\frac{1}{4}$  in. wide collar was at one end of the block. Two vertical holes, 2.5 in. long and 10 cm. in diameter were drilled in the block. The block was heated by a 9 in. by 8 in. electric heating shell which was encased in aluminum. The deposit was placed in a Pyrex heating boat which was 1 in. tall and 10 cm. in diameter. Air was metered through a rotameter and jetted onto the deposit through a steel hypodermic needle. The needle extended  $2\frac{1}{2}$  inches inside the drilled hole. The temperature was found by means of a Chromel-Alumel thermocouple, which extended into the deposit.

In a typical experiment 0.2 g. of deposit was placed in a Pyrex boat and packed lightly into the Pyrex container. The thermocouple was placed in the deposit and air introduced at the rate of 200 cc./min. The variac which controlled the heating rate was set at 80 volts and was kept at this reading through the experiment. Temperature readings were taken every 10 minutes until 40 minutes had elapsed. After 40 minutes readings were taken in 0.5 or 1.0 minute intervals, and the degree centigrade resulting from a sudden increase in temperature was taken as the glow point of the deposit. Table II lists the average glow point of deposits containing compounds of this invention.

Table II

| Additive: | Average glow point, ° C. |
|-----------|--------------------------|
| BCPMP     | 320                      |
| BCPPP     | 325                      |
| BCPMTP    | 324                      |
| TCP       | 327                      |
| None      | 309                      |

Table II shows that the compounds of this invention raise the glow point or ignition temperature of the deposits.

The novel additives of the present invention may be used in conjunction with the previously mentioned halohydrocarbons. Examples of these halohydrocarbons are ethylene dibromide or dichloride, acetylene tetrabromide, 2,2,3-trichlorobutane, 2-chloro 2,3-dibromobutane, and the dibromotoluenes. Mixtures of these halohydrocar-

bons, such as a mixture of ethylene dibromide and ethylene dichloride, may also be used. In general halohydrocarbons having a vapor pressure in the range of 0.1 mm. to 100 mm. mercury at 50° C. are capable of being used.

5 It is desirable that the combined organophosphorus and halohydrocarbons contain not more than about 90% by weight of the halohydrocarbons.

In general, the quantity of additives required in the fuel is that necessary to convert (theoretically) all the lead

10 present as tetraalkyl lead into the corresponding lead halide and lead salt of the phosphonite or thionophosphate concerned. Such a quantity is usually referred to as "1 theory." Greater or smaller quantities may be employed in some circumstances depending upon the par-

15 ticular components of the fuel and the type of engine in which it is intended to be used. In fact one of the merits of the present invention is that it allows greater variation in the quantity of additive employed than is permissible when a halohydrocarbon is used as the sole additive.

20 Even small excesses of halohydrocarbon additives are detrimental in such circumstances whereas with the additives of this invention a substantial excess can be tolerated without adverse results. The preferred range of total additive content of the fuel is from 0.9 to 1.2 theories.

25 Both the fuels and the compositions suitable for addition to fuels provided by this invention may advantageously contain further compounds known to exert a stabilizing and/or antioxidant effect on hydrocarbons of the gasoline boiling range. In this connection, 2,4-dimethyl-6-

30 tertiary butyl phenol is a particularly useful additive, other compounds such as hydroquinone, 2,6-ditertiary-butyl-4-methyl phenol, N-phenyl- $\alpha$ -naphthylamine and N,N'-ditertiary-butyl-p-phenylenediamine may be employed.

The fuels of this invention may be compounded by

35 simply mixing the ingredients in any order. Thus the organophosphorus additive may be added to a leaded gasoline which already contains a halohydrocarbon additive. Alternatively, the organophosphorus may be incorporated in a tetra-alkyl lead fluid containing a halohydro-

40 carbon additive and whole composition blended into the fuel. Again the organo-phosphorus additive may be added to an unleaded gasoline and the tetra-alkyl lead fluid containing a halohydrocarbon scavenger added subsequently.

45 Pursuant to the requirements of the patent statutes, the principle of this invention has been explained and exemplified in a manner so that it can be readily practiced by those skilled in the art, such exemplification including what is considered to represent the best embodiment of

50 the invention. However, it should be clearly understood that, within the scope of the appended claims, the invention may be practiced by those skilled in the art, and having the benefit of this disclosure, otherwise than as specifically described and exemplified herein.

55 That which is claimed as patentably novel is:

1. A composition of matter represented by the formula:



60 in which R is selected from the group consisting of hydrogen and lower alkyl and phenyl radicals; Y is selected from the group consisting of lower alkyl and phenyl radicals and n is an integer from 1 to 2 inclusive.

70 2. As a new composition of matter, bis(betachloropropyl)methyl phosphonite.

3. As a new composition of matter, bis(betachloropropyl)phenyl phosphonite.

4. As a new composition of matter, bis(betachloropropyl)methyl thionophosphonate.

75

5. A method of preparing the halogenated thiono esters of primary phosphonic acids of the formula



wherein R is selected from the group consisting of hydrogen and lower alkyl and phenyl radicals and Y is selected from the group consisting of lower alkyl and phenyl radicals, which comprises reacting the corresponding halo-  
ester of phosphorous acid and sulphur and thereby pro-  
ducing said halogenated thiono ester of a primary phos-  
phonic acid.

6. A method of preparing the halogenated thiono esters

of primary phosphonic acids in accordance with claim 5, in which the haloester of phosphorous acid is bis(beta-chloropropyl)methyl phosphonite.

References Cited in the file of this patent

UNITED STATES PATENTS

|           |                |                |
|-----------|----------------|----------------|
| 2,405,560 | Campbell       | Aug. 13, 1946  |
| 2,427,173 | Withrow        | Sept. 9, 1947  |
| 2,460,043 | Teeters        | Jan. 25, 1949  |
| 2,653,161 | Ballard et al. | Sept. 22, 1953 |

OTHER REFERENCES

Kosolapoff: Organo Phosphorus Compounds, page 185  
1950), John Wiley & Sons, Inc., New York, N.Y.